

147

Patented May 20, 1930

1,759,635

## UNITED STATES PATENT OFFICE

KARL B. THEWS, OF DREXEL HILL, AND JOSEPH S. CARLITZ, OF PHILADELPHIA,  
PENNSYLVANIA; SAID CARLITZ ASSIGNOR TO SAID THEWS.

## TREATMENT OF IRON OR STEEL

No Drawing.

Application filed December 7, 1929. Serial No. 412,565.

This invention relates to a process for reducing the dissolution of iron and steel during the removal of iron oxide or scale in pickling baths of sulphuric or other acids. The methods disclosed herein are also useful in preventing corrosion of iron and steel containers of such acids.

Heretofore it has been customary to use various inhibiting agents in the pickling baths to prevent pitting or etching of the surface of the iron or steel. These substances have been more or less successful in the attainment of such results, the best of these inhibitors so far used apparently being the substitution products of normal thiourea of which the ditolyl derivatives are the most effective.

We have discovered that the normal selenourea and normal tellurourea derivatives are generally superior to the corresponding derivatives of normal thiourea in preventing the solution of iron or steel in acidic liquids such as pickling baths. The use of such derivatives is claimed in an application Serial Number 412,565, filed of even date herewith.

We have further found, however, that derivatives of pseudo-thiourea, pseudo-selenourea, and pseudo-tellurourea are equivalent or superior as inhibitors to the corresponding derivatives of normal thiourea, normal selenourea and normal tellurourea. It is accordingly the object of the present invention to improve the processes heretofore used by the use as inhibitors of the derivatives of the above mentioned pseudo-ureas.

The attainment of the object outlined above and more specific objects of the invention will be clear from the following description.

The pseudo-derivatives which are found to have the more effective inhibiting action have the following general formula:



in which X represents sulphur, selenium, or tellurium, R represents hydrogen, or an alkyl, aryl or acyl group, and R' represents an alkyl, aryl or acyl group; this definition including substances having the same general formula in which a bivalent alkyl, aryl or acyl sub-

stituent group, such as an ethylene group, replaces R' and an R, being connected to both a nitrogen atom and the X atom.

As examples of suitable alkyl groups, there may be cited methyl, ethyl, propyl, butyl, aryl, etc., propyl, butyl, aryl and higher radicals being of any of the various isomeric types, such as normal, iso-, tertiary, etc. Substituted alkyl groups may also be used, in which, for example, one or more hydrogen atoms are replaced by amino, sulphonic, nitro, or other groups.

The aryl groups may be joined to the nitrogen or X atoms either at the nucleus or side chain. Of the first type, phenyl, tolyl, xylyl, or naphthyl, etc. are examples. The junction to the nitrogen or sulphur, selenium or tellurium atoms may take place at any of the unsubstituted carbon atoms. Of the second type, benzyl is the best example. Here again there may be various groups replacing the hydrogen atoms in either the nucleus or side chains.

The acyl groups may be formyl, acetyl, propionyl, benzoyl, phthalyl, succinyl, etc., or substituted derivatives thereof.

If two substituent groups are present there may be obtained (n,  $\psi$ ), or ( $\psi$ , v) derivatives. In view of the fact that the substituted positions are not symmetrical, two different substituent groups may form two different n,  $\psi$ , etc. derivatives. For example, n-methyl  $\psi$ -benzyl selenourea is different from  $\psi$ -methyl n-benzyl selenourea.

Similar considerations will indicate the numerous isomeric derivatives producible by the presence of either three or four substituents. The presence of stereoisomers is readily explainable by reference to the structural formula.

There may also be used derivatives in which one of the nitrogen atoms and the X atom are joined to a single radical, each by a single linkage whereby a cyclic compound is obtained. The radicals in these cases may be either alkyl, aryl, or acyl.

It will be understood that where the term "alkyl" is used, it is in a broad sense so as to include not only the alkylene groups, such as ethylene, but also heterocyclic derivatives

such as terpene groups. The terms "aryl" and "acyl" are intended to have similar broad interpretations, the term "aryl", for example, being intended to include "aralkyl" such as benzyl.

- 5 Of the various derivatives pointed out above  $\psi$ -benzyl thiourea is found to have a very efficient inhibiting action. Furthermore it is very readily prepared by treatment of 10 normal thiourea in alcoholic solution with benzyl chloride with the application of heat. A rearrangement of the molecular structure takes place during such reaction whereby a pseudo derivative is formed.
- 15 In a general way it may be said that the operative substances are represented by the general formula above in which one or more of the R's represent an organic radical or hydrogen, and in which X represents S, Se 20 or Te. It appears that the inhibiting action to a greater or less degree is characteristic of this class of compounds.

The mechanism of the process involved in using these substances is similar to that 25 usually used. The pickling solution may contain sulphuric or other suitable acidic materials such as are now used in effective concentrations. For example, approximately 10% sulphuric acid solution in water may 30 be used. To such pickling solution up to approximately 1% of one of the inhibiting agents is added. The pickling is then effected in the usual fashion by submerging the iron or steel articles in the solution either 35 at ordinary or elevated temperatures. In cases where it is desired to protect a tank against acid which is contained therein, the inhibiting agent is added to the acid.

Of the various derivatives the alkyl and 40 aryl are generally found to be best; the acyl derivatives are less effective. The best derivatives appear to be those in which a substituent group is attached to the X atom in the  $\psi$  position, although operative inhibitors 45 are obtained if the substituent group or groups enter the n and v positions. In general the pseudo-thio-, seleno-, and telluro-derivatives are either equivalent or superior 50 to the normal derivatives containing similar substituents. Of the three groups, the pseudo-thiourea derivatives appear most effective.

For convenience in handling the inhibiting substances in the small quantities necessary 55 in a pickling bath, it may be desirable to mix them with a large proportion of a carrier substance which may be of such nature as to assist the pickling action, for example, sodium chloride or sodium bisulphate. Mixtures of various inhibiting agents may also be used.

The various derivatives referred to are best prepared by the general methods well known to the art. In general it may be stated that 60 the seleno- and tellurourea derivatives are

prepared similarly to the corresponding pseudo-thiourea derivatives although special methods of preparation are well known to the art. In view of the fact that the preparations of the derivatives form no part of the instant invention, they have not been discussed in detail.

What we claim and desire to protect by Letters Patent is:

1. An aqueous solution of a non-oxidizing acid capable of dissolving iron oxides to which has been added an inhibitor comprising an organic pseudo-substitution product of  $\text{NH:C(XH)-NH}_2$ , in which X represents S, Se or Te. 75
2. An aqueous solution of a non-oxidizing acid capable of dissolving iron oxides to which has been added an inhibitor comprising an organic pseudo-substitution product of thiourea. 80
3. An aqueous solution of a non-oxidizing acid capable of dissolving iron oxides to which has been added an inhibitor comprising an organic pseudo-substitution product of  $\text{NH:C(SH)-NH}_2$ , in which the hydrogen attached to sulphur is replaced by an alkyl, 90 aryl, or acyl group. 95
4. An aqueous solution of a non-oxidizing acid capable of dissolving iron oxides to which has been added an inhibitor comprising a substance having the general formula  $\text{NR:C(SR')-NR}_2$ , in which R represents hydrogen or an alkyl, aryl or acyl group, and R' represents an alkyl, aryl or acyl group. 100
5. An aqueous solution of a non-oxidizing acid capable of dissolving iron oxides to which has been added an inhibitor comprising  $\psi$ -benzyl thiourea. 105
6. The process of pickling iron and steel products which consists in treating said products with an aqueous solution of a non-oxidizing acid capable of dissolving iron oxides to which has been added an inhibitor comprising an organic pseudo-substitution product of  $\text{NH:C(XH)-NH}_2$ , in which X represents S, Se or Te. 110
7. The process of pickling iron and steel products which consists in treating said products with an aqueous solution of a non-oxidizing acid capable of dissolving iron oxides to which has been added an inhibitor comprising an organic pseudo-substitution product of thiourea. 115
8. The process of pickling iron and steel products which consists in treating said products with an aqueous solution of a non-oxidizing acid capable of dissolving iron oxides to which has been added an inhibitor comprising an organic pseudo-substitution product of  $\text{NH:C(SH)-NH}_2$ , in which the hydrogen attached to sulphur is replaced by an alkyl, 120 aryl or acyl group. 125
9. The process of pickling iron and steel products which consists in treating said products with an aqueous solution of a non-oxidizing acid capable of dissolving iron oxides to which has been added an inhibitor comprising an organic pseudo-substitution product of  $\text{NH:C(XH)-NH}_2$ , in which X represents S, Se or Te. 130

147

1,759,635

ing acid capable of dissolving iron oxides to which has been added an inhibitor comprising a substance having the general formula  $NR:C(SR')-NR_2$ , in which R represents hydrogen or an alkyl, aryl or acyl group, and R' represents an alkyl, aryl or acyl group.

10. The process of pickling iron and steel products which consists in treating said products with an aqueous solution of a non-oxidizing acid capable of dissolving iron oxides to which has been added an inhibitor comprising  $\gamma$ -benzyl thiourea.

In testimony of which invention, we have hereunto set our hands, at Philadelphia, Pennsylvania, on this 6th day of December, 1929.

KARL B. THEWS.  
JOSEPH S. CARLITZ.

20

25

30

35

40

45

50

55

60

65